

3,232,779

METHODS OF PRODUCING REGENERATED  
CELLULOSE

Nikolaus Augustin Schönfeldt, Molndal, and Kurt Helmut Grunewald, and Olof Rune Steijner, Goteborg, Sweden, assignors to Mo Och Domsjö Aktiebolag, Örnsköldsvik, Sweden, a corporation of Sweden

No Drawing. Filed Nov. 20, 1959, Ser. No. 854,219  
Claims priority, application Sweden, Jan. 20, 1955,

543/55

5 Claims. (Cl. 106—165)

This application is a continuation-in-part of our co-pending application Serial No. 559,749, filed on January 17, 1956, and now abandoned.

The present invention relates to the production of regenerated cellulose, and is most particularly concerned with the use of certain substances as additives in various steps of the production of regenerated cellulose.

Regenerated cellulose is produced by converting cellulose to a soluble compound thereof and in a subsequent step reforming the cellulose. The most widely used process of producing regenerated cellulose is the viscose process in which the cellulose is converted to cellulose xanthate. Briefly described, this process comprises mercerizing cellulose with caustic soda to produce alkali cellulose. After squeezing out excess soda, the alkali cellulose is comminuted in a mill and is then stored for a period of time to undergo aging. Thereupon, carbon disulfide is introduced whereby cellulose xanthate is formed. The cellulose xanthate is dissolved in dilute alkali to form a viscous solution called viscose. The viscose is filtered and stored for a few days whereupon it is extruded through fine holes in spinnerets into a spinning bath, which usually comprises sulfuric acid and various salts. Thereby, the viscose is coagulated and solidified with reformation of the cellulose in the form of filaments or fibers, which are subjected to washing and other treatments and is then dried. The viscose may also be extruded through dies adapted to form films, whereby the regenerated cellulose will be obtained in film form. Regenerated cellulose can also be prepared by the cuprammonium process, which is similar to the viscose process, but uses a solution of cuprammonium hydroxide to dissolve the cellulose. The processes of producing regenerated cellulose are well-known and described in the technical and patent literature, and will not be described in detail here.

In various steps of the production of regenerated cellulose various substances are used as additives. These serve the purpose of facilitating and improving the process of production in various respects. Depending on which object the additives have to fulfill, they may be entirely different in their chemical constitution and properties. The additives are used for example to improve the filtering characteristics of the viscose, to prevent yarn milkiness, to reduce the gel swelling during the spinning or as anti-clogging agents or as finishing agents (avivage agents) to soften the finished fiber, etc. Additives are used not only in the production of viscose rayon but also in the production of cuprammonium rayon.

Generally, different products are used in different steps of the production process and consequently their solubility in the viscose or in the spinning bath may be quite different. If the product is added to the viscose it is desirable that the substance in question dissolves clearly therein. If the product is added to the spinning bath it is advantageous if it dissolves clearly or is finely dispersed therein. It is frequently found that products which are added to the viscose are not sufficiently soluble in the spinning bath and vice versa. It would of course be

highly advantageous to be able to employ products which are soluble or dispersible both in the viscose and in the spinning bath and thereby can beneficially influence the process of production. If on the other hand, the agents are used to soften rayon silk or rayon staple fibers as such or in combination with other substances, it is important that finely dispersed emulsions can be used so that softening of the fibers occurs evenly.

A further circumstance which is to be considered is the chemical resistance of the additives in various stages of the process. When adding it prior to spinning, it will be subjected to alkalies, in the spinning bath it is exposed to sulfuric acid and to salts at an elevated temperature. If the agent in question is resistant to alkali, but is attacked in the spinning bath by sulfuric acid or the salts present in the spinning bath, precipitates may be formed which may affect the spinning process adversely. In addition the action of the spinning bath becomes still stronger in the evaporation of the spinning bath, which often takes place at 80° or higher temperatures, so that decompositions of the additives may occur, which may result in considerable losses in economy.

The present invention relates to a method of preparing regenerated cellulose, which includes the use as additives in any stage of the production, including finishing, of regenerated cellulose of compounds selected from the group consisting of alkylene oxide adducts of polyamines of the general formula



in which R represents hydrocarbon radical having from 6 to 22 carbon atoms, x is 1 to 5, and z is 2 to 3. The compounds used according to this invention are ethylene oxide and propylene oxide adducts of said polyamines, wherein the number of ethylene oxide or propylene oxide units is from 1 to 10. These compounds are used in amounts ranging from 0.1 to 4% by weight based on the cellulose.

The radical R may be, e.g., an aliphatic straight-chain or branched-chain, saturated or unsaturated hydrocarbon grouping. Representative examples include ethylhexyl, dodecyl, hexadecyl, octadecenyl and octadecyl groups. Furthermore, R may be an aryl or alkylaryl or aralkyl group. Examples include dodecylbenzene, octadecylbenzene and nonylnaphthalene groups.

Compounds of the above type may be obtained by condensing an appropriate polyamine (such as, e.g., ethylene diamine, diethylene triamine, triethylene tetramine, di-propylene triamine, ethyl dipropylene triamine etc., or mixtures of such polyamines) with a compound containing the radical R linked to a reactive group, such as halogen, and then condensing the substances thus obtained with an alkylene oxide, such as ethylene oxide or propylene oxide to introduce into the compound one or more alkylene oxide units per mole of the compound. Since the nitrogen atoms of the resulting compounds are linked only to carbon atoms, these compounds are chemically very resistant even after addition of the alkylene oxide.

By a suitable choice of the hydrocarbon radical R, of the number of nitrogen atoms equal to or above 2 and the number of alkylene oxide units per mole of compound it is possible to prepare substances which are most suitable as additive either in the production or in the finishing of the regenerated cellulose. The above mentioned possibilities of varying the composition permit, in addition to a suitable adaptation of functional properties the preparation of compounds having good solubility and dispersibility characteristics in various stages of the process of producing regenerated cellulose.

If the compounds are to be used as finishing agents the radical R in the above formula should preferably be

a saturated group comprising 12-22 carbon atoms, and more preferably 18-22 carbon atoms, the number of nitrogen atoms should preferably be within the range of from 2 to 4 ( $x=1$  to 3) and the polyglycol residue should preferably be relatively short, e.g., from 1 to 6 alkylene oxide units.

If the compounds are to be used as additives in various stages of the production, e.g., be added to the spinning bath or the viscose or even earlier in the process, the radical R contains preferably 12-22 carbon atoms, more preferably 18-22 carbon atoms, and may advantageously be an unsaturated group, the number of nitrogen atoms should preferably be within the range of from 2 to 6 ( $x=1$  to 5) and the polyglycol group should preferably be relatively long and contain 6 to 10, e.g., 8 alkylene oxide units.

Experiments have proved that, e.g., a compound of the above type, in which R was an octadecenyl group, the amino groups were derived from a mixture of polyethylene polyamines, substantially from diethylene triamine to tetraethylene pentamine, and which compound finally contained about 10 ethylene oxide units per molecule is an efficient sulfur dispersing agent. If a sulfur dispersion is prepared in a solution which contains 7% sulfuric acid, 4.5% zinc sulfate and 16% sodium sulfate by adding thereto a sodium thiosulfate solution, this becomes progressively more cloudy when permitted to stand. If a control sample without additive shows an initial light transmission of 100% and this transmission of light decreases in 3 minutes to 50%, this period may be increased to about 30 minutes, i.e. about 10 times, by adding 1 g. of the above compound.

Compounds of the above formula may exhibit marked surface-active properties, resulting in a decrease in the surface tension of the viscose and the spinning bath. By varying the radical R, the polyamines used and the amount of ethylene oxide, the surface tension reduction can be kept within suitable limits.

In compounds of the above type, at least one of the nitrogen atoms can be quaternized by treatment with, e.g., dimethyl sulfate, diethyl sulfate, ethyl chloride etc. The compounds can also be condensed with formaldehyde or acetic anhydride to increase their stability to light. Quaternized compounds as well as such formaldehyde and acetic anhydride condensation products are within the ambit of this invention.

The amount of additive to be employed in the production of regenerated cellulose can vary to a relatively large extent. In the case of adding it in the mill, an amount of 0.1 to 0.4% based on the weight of cellulose, is often sufficient, in the case of adding it to the viscose, preferably 0.3 to 0.5 g./l. will be used. As an additive to the spinning bath, it is customary to use 1 to 4 gs. per kg. of fiber. As an "all skin agent" an addition of 1 to 3 gs. per liter of viscose is advantageous. The term "all skin agent" (also called "greening agent") denotes a substance, the action of which is that the fiber throughout its cross-section is imparted the properties which normally are present in its surface (skin). Such additives reduce the gel swelling. When softening regenerated cellulose, an amount of softening agent, in the case of rayon staple fiber, of 0.4 to 0.5%, and in the case of rayon filaments 0.7 to 0.8% is often advantageous.

The substance of the present invention may be used in the form of the pure compounds, but it is also possible to employ mixtures containing two or more compounds of the above formula.

The invention is illustrated but not limited by the following examples:

#### Example 1

1 mole of ketyl chloride obtained by chlorination of kerosene is reacted at 150 to 160° C. with 1.2 moles of diethylene triamine whereupon the product is condensed with 8 moles of ethylene oxide, 2 gs. of this product per

kg. of finished yarn added to the spinning bath improves the spinning properties (e.g., less slubbing, prevention of spinneret incrustation) considerably.

#### Example 2

One mole of cocoa fat chloride obtained from cocoa fat alcohol by replacing the hydroxyl group by chlorine, is reacted with 5 moles of ethylene diamine under reflux in a solution of 2000 mls. of absolute ethanol for 4 hours, whereupon the ethanol is distilled off. The residue separates into two layers. The top layer which contains the product is decanted. 1000 mls. of water are added and the white precipitate extracted with ether. The ethereal extract is dried over anhydrous sodium sulfate and the solution is evaporated. The product is condensed with 6 moles of ethylene oxide. One gram of this product per liter of viscose reduces swelling of the gel fiber and counteracts effectively the formation of milky yarn.

#### Example 3

204 gs. of dodecyl chloride is reacted at 160° C. with 200 gs. of polyethylene polyamines obtained as distillation residue after distilling off diethylene triamine and triethylene tetramine from a polyethylene polyamine mixture obtained by reaction of ethylene dichloride and ammonia. The reaction is complete after 3 hours. The resulting product is condensed with 6 moles of ethylene oxide, 1 g. of this product per liter of viscose reduces swelling of the gel fiber.

#### Example 4

Ketyl benzene is reacted in a known manner with formaldehyde and gaseous hydrogen chloride in the presence of zinc chloride to form ketyl phenyl chloride. 500 parts by weight of this substance are reacted with 200 parts by weight of polyamines in accordance with Example 3. Thereupon 10 moles of ethylene oxide are condensed with the resulting product. An addition of 0.5 g. per liter of spinning bath improves the extrusion of the viscose and prevents the spinneret incrustation.

As above stated, compounds of the above types can be quaternized, e.g., with dimethyl sulfate, ethyl chloride, benzyl chloride etc. They can also, if desired, be treated with formaldehyde or acetic anhydride especially if the product is to be used as a finishing agent, in order to improve their resistance to light. Thereby formyl or acetyl groups are linked to certain of the nitrogen atoms. As examples of such agents, the following may be mentioned.

#### Example 5

1 mole of octadecyl chloride is condensed with 4 moles of dipropylene triamine at 155° C. for 5 hours. Thereupon 1 mole of sodium hydroxide is introduced, whereupon excess of dipropylene triamine is distilled off. The octadecyl dipropylene triamine is then reacted with 2 moles of ethylene oxide. Thereupon the product is reacted with 1 mole of acetic acid anhydride at elevated temperature. If rayon fiber is softened with this product, the properties in the subsequent spinning and weaving steps can be substantially improved.

#### Example 6

1 mole of dodecyl tetraethylene pentamine is condensed with 6 moles of propylene oxide. 5 gs. of this product per liter of bath are used to soften rayon staple fiber.

#### Example 7

1 mole of 9,10-octadecenyl chloride is reacted at 150° C. with 4 moles of triethylene tetramine. When the reaction is completed, 1 mole of sodium hydroxide is added to neutralize the hydrogen chloride formed, whereupon excess of triethylene tetramine is distilled off, suitably under vacuum. After separating sodium chloride precipitated 5 moles of ethylene oxide are reacted with the product. The 9,10-octadecenyl triethylene tetramine polyethylen

polyglycol ether is then quaternized with 2 moles of dimethyl sulfate. 0.4 g. of this product per liter of viscose improves the filtering properties.

What we claim is:

1. A process for producing regenerated cellulose from cellulose which includes the step of using as an additive, in any stage of the process, an amount within the range from about 0.1 to about 4% by weight, based on the cellulose, of a compound selected from the group consisting of (1) the reaction product of (a) from about one to about ten moles of an alkylene oxide having from two to three carbon atoms with (b) one mole of at least one polyamine having the formula:



in which R is a hydrocarbon radical having from about six to about twenty-two carbon atoms, z is an integer from 2 to 3, and x is a number from 1 to 5; (2) reaction products of (1) a quaternizing agent selected from the group consisting of lower alkyl and benzyl quaternizing agents; and (3) reaction products of (1) with a member selected from the group consisting of formaldehyde and acetic anhydride.

2. A process for producing regenerated cellulose from cellulose which includes the step of using as an additive, in any stage of the process, an amount within the range from about 0.1 to about 4% by weight, based on the cellulose, of the reaction product of (a) from about one to about ten moles of an alkylene dioxide having from two to three carbon atoms with (b) one mole of at least one polyamine having the formula:



in which R is a hydrocarbon radical having from about six to about twenty-two carbon atoms, z is an integer from 2 to 3, and x is a number from 1 to 5.

3. A viscose spinning solution containing from about 3% to about 4%, based on the weight of the cellulose in the viscose, of a modifier corresponding to the formula



wherein R is a fatty alkyl hydrocarbon chain having be-

tween 8 and 18 carbon atoms, n is a whole number of at least 2 but not greater than 3, x, y and z are whole numbers and the sum of x, y and z is about 10.

4. A viscose spinning solution containing from about 0.1 to about 4% by weight of the cellulose in the viscose of a modifier selected from the group consisting of (1) the reaction product of (a) from about one to about ten moles of an alkylene oxide having from two to three carbon atoms with (b) one mole of at least one polyamide 10 having the formula:



in which R is a hydrocarbon radical having from about 15 six to about twenty-two carbon atoms, z is an integer from 2 to 3, and x is a number from 1 to 5; (2) reaction products of (1) with a quaternizing agent selected from the group consisting of lower alkyl and benzyl quaternizing agents; and (3) reaction products of (1) with a member selected from the group consisting of formaldehyde 20 and acetic anhydride.

5. A viscose spinning solution containing from about 0.1 to about 4% by weight of the cellulose in the viscose, as a modifier, of the reaction product of (a) from about 25 one to about ten moles of an alkylene oxide having from two to three carbon atoms with (b) one mole of at least one polyamine having the formula:



in which R is a hydrocarbon radical having from about 30 six to about twenty-two carbon atoms, z is an integer from 2 to 3, and x is a number from 1 to 5.

#### References Cited by the Examiner

##### UNITED STATES PATENTS

|    |           |        |                  |         |
|----|-----------|--------|------------------|---------|
| 35 | 2,593,466 | 4/1952 | MacLaurin et al. | 106—165 |
|    | 2,674,619 | 4/1954 | Lundstred        | 260—584 |
|    | 2,759,975 | 8/1956 | Chiddix et al.   | 106—165 |
|    | 2,792,281 | 5/1957 | Castellan        | 106—165 |
| 40 | 2,852,333 | 9/1958 | Cox et al.       | 106—165 |

MORRIS LIEBMAN, Primary Examiner.

JOSEPH R. SPECK, Examiner.

A. LIEBERMAN, Assistant Examiner.

UNITED STATES PATENT OFFICE  
CERTIFICATE OF CORRECTION

Patent No. 3,232,779

February 1, 1966

Nikolaus Augustin Schönfeldt et al.

It is hereby certified that error appears in the above numbered patent requiring correction and that the said Letters Patent should read as corrected below.

Column 1, line 16, for "mort" read -- more --; column 2, line 64, for "additive" read -- additives --; column 3, line 28, for "intial" read -- initial --; line 64, for "substance" read -- substances --; column 5, line 29, for "dioxide" read -- oxide --.

Signed and sealed this 31st day of January 1967.

(SEAL)

Attest:

ERNEST W. SWIDER

Attesting Officer

EDWARD J. BRENNER

Commissioner of Patents